

# United States Patent [19]

Takahashi et al.

[11] Patent Number: 5,008,236

[45] Date of Patent: Apr. 16, 1991

## [54] HEAT-SENSITIVE RECORDING MATERIAL

[75] Inventors: Yoshiyuki Takahashi, Kawasaki; Kunitaka Toyofuku, Sakura; Akiko Iwasaki, Urawa, all of Japan

[73] Assignee: Oji Paper Co., Ltd., Tokyo, Japan

[21] Appl. No.: 458,191

[22] Filed: Dec. 28, 1989

## [30] Foreign Application Priority Data

Apr. 5, 1989 [JP] Japan ..... 1-84788

[51] Int. Cl.<sup>5</sup> ..... B41M 5/18

[52] U.S. Cl. ..... 503/209; 503/208;  
503/225

[58] Field of Search ..... 427/150-152;  
503/208, 209, 225

## [56] References Cited

### U.S. PATENT DOCUMENTS

4,539,578 9/1985 Igarashi et al. ..... 503/207  
4,882,311 11/1989 Ikeda et al. ..... 503/208

### FOREIGN PATENT DOCUMENTS

3703479 8/1987 Fed. Rep. of Germany ..... 503/209  
58-72499 4/1983 Japan ..... 503/209  
59-133094 7/1984 Japan ..... 503/209  
59-133095 7/1984 Japan ..... 503/209  
61-50936 3/1986 Japan ..... 503/209  
62-251186 10/1987 Japan ..... 503/209

## OTHER PUBLICATIONS

Patent Abstracts of Japan, vol. 7, No. 165, Jul. 20, 1983,  
JP-A-58 72499.

Patent Abstracts of Japan, vol. 12, No. 126, Apr. 1988,  
JP-A-62 251186.

Patent Abstracts of Japan, vol. 10, No. 208, Jul. 22,  
1986, JP-A-61 50936.

Patent Abstracts of Japan, vol. 8, No. 262, Nov. 30,  
1984, JP-A-59 133095.

Patent Abstracts of Japan, vol. 8, No. 262, Nov. 30,  
1984, JP-A-59 133094.

Spengler, G. et al, "Über die Synthese Ausgewählter  
Polyphenyläther und deren Eignung als Schmieröle",  
*Deutsche Luft- und Raumfahrt, Forschungsbericht*  
68-86 (Dec. 1968), pp. 1-51.

Primary Examiner—Bruce H. Hess

Attorney, Agent, or Firm—Armstrong, Nikaido,  
Marmelstein, Kubovcik & Murray

## [57] ABSTRACT

A heat-sensitive recording material with an excellent  
recording sensitivity and capable of recording thereon  
high quality images at a high recording speed, comprising  
a heat-sensitive color-forming layer formed on a  
substrate sheet and comprising a colorless dye precursor,  
a color-developing agent, a binder and a sensitizing  
agent consisting essentially of 1,2-diphenoxylbenzene.

6 Claims, No Drawings

## HEAT-SENSITIVE RECORDING MATERIAL

## BACKGROUND OF THE INVENTION

## 1. Field of the Invention

The present invention relates to a heat-sensitive recording material. More particularly, the present invention relates to a heat-sensitive recording material which has a high whiteness and an enhanced recording property at a high speed.

## 2. Description of the Related Art

Heat-sensitive recording materials in which a heat color-developing reaction of a colorless or light colored leuco dye with an organic acid material, for example, a phenol compound or organic acid compound, is utilized, are disclosed by, for example, Japanese Examined Patent Publication (Kokoku) Nos. 43-4160, 45-14039 and 48-27736.

These heat-sensitive recording materials are advantageous in that colored images can be easily formed only by heating and the recording apparatus can be made relatively compact and small size, and thus are widely utilized as information-recording materials. Also, facsimile machines and printers for which the heat-sensitive recording materials are used, have been greatly improved to an extent such that the formation of colored images at a very high speed, considered impossible or very difficult in the past, is now possible.

Due to the above-mentioned development of the high speed heat-sensitive recording machines, the heat-sensitive material to be used for the high speed recording machines must have an enhanced recording sensitivity, in comparison with conventional heat-sensitive recording materials, and many attempts have been made to meet the above-mentioned requirement. Most of these attempts relate to combinations of specific leuco dyes with the color developing agents, or to utilization of specific heat-fusible substances.

The heat-fusible substances are used as a sensitizing agent for the color-developing reaction in the heat-sensitive color forming layer and include, for example, the phenyl 1-hydroxy-2-naphthoate disclosed in Japanese Unexamined Patent Publication No. 57-191089, p-benzyl-biphenyl disclosed in Japanese Unexamined Patent Publication No. 60-82382, benzyl naphthyl ether disclosed in Japanese Unexamined Patent Publication No. 58-87094, dibenzyl terephthalate disclosed in Japanese Unexamined Patent Publication No. 58-98285, benzyl p-benzyloxybenzoate disclosed in Japanese Unexamined Patent Publication No. 57-201691, diphenyl carbonate and ditolyl carbonate disclosed in Japanese Unexamined Patent Publication No. 58-136489, m-terphenyl disclosed in Japanese Unexamined Patent Publication No. 57-89994, 1,2-bis(m-tolyl)ethane disclosed in Japanese Unexamined Patent Publication No. 60-56588, and 1,5-bis(p-methoxyphenoxy)-3-oxapentane disclosed in Japanese Unexamined Patent Publication No. 61-58789.

When a heat-sensitive color-forming layer containing the heat-fusible sensitizing agent is heated, first the sensitizing agent is melted and the leuco dye and the color-developing agent are dissolved in the melt, whereby the molecule of the dissolved leuco dye and color-developing agent are mixed and reacted with each other to develop a color in the color-forming layer.

Therefore, the heat-fusible sensitizing agent must have a proper melting point, preferably from 80° C. to

110° C., and be compatible with the leuco dye and the color developing agent.

Also, preferably the heat-fusible sensitizing agent does not cause a lowering of the whiteness of the heat sensitive color developing layer. Therefore, the heat-fusible sensitizing agent must be substantially forming layer.

When a certain type of conventional heat fusible sensitizing agent is contained, a white powder-like substance appears on the resultant color-forming layer, with a lapse of time; which is known as the color-forming layer whitening phenomenon. The whitening phenomenon is believed to depend closely on the sublimating property of the heat-fusible sensitizing agent, and therefore, the heat-fusible sensitizing agent must have no or a very low sublimating property.

In a practical recording operation, frequently the heat sensitive recording materials are temporarily exposed to a high temperature of about 60° C. to about 0° C. Under such a condition, the heat-sensitive color-forming layer must exhibit a high heat stability and must not develop a color at the above-mentioned temperature. Therefore, the heat fusible sensitizing agent must not affect the heat stability of the heat-sensitive color-forming layer.

As stated above, many heat fusible sensitizing agents have been provided, but very few can meet all of the above-mentioned requirements, and thus a new type of heat fusible sensitizing agent is urgently required.

## SUMMARY OF THE INVENTION

An object of the present invention is to provide a heat-sensitive recording material which has an enhanced recording sensitivity, a satisfactory whiteness and resistance to the whitening phenomenon, and does not affect the heat stability of the heat-sensitive color-forming layer, and thus is useful for recording high quality clear colored images, under high speed recording conditions.

This object can be attained by the heat-sensitive recording material of the present invention, which comprises a substrate sheet and a heat-sensitive color-forming layer formed on at least one surface of the substrate sheet and comprising a substantially colorless dye precursor, a color developing agent reactive with the dye precursor upon heating, to develop a color, and a binder, said heat-sensitive color-forming layer further comprising a sensitizing agent consisting essentially of 1,2-diphenoxylbenzene of the formula (I):



## DESCRIPTION OF THE PREFERRED EMBODIMENTS

In the heat-sensitive recording material of the present invention, the heat-sensitive color-forming layer must contain, in addition to a dye precursor, a color developing agent, and a binder, a sensitizing agent consisting essentially of 1,2-diphenoxylbenzene of the formula (I).

The inventors of the present invention discovered that the compound of the formula (I) having a melting point of 92° C. effectively and significantly enhances the recording sensitivity and heat stability of the heat-sensitive color-forming layer, without affecting the whiteness of the color developing layer or causing an undesirable whitening of the color developing layer, whereas the conventional heat fusible sensitizing agent consisting of a higher fatty acid amide, for example, stearylamide or palmitylamide, causes an unsatisfactory recording sensitivity of the resultant color-forming layer.

The reasons why the compound of the formula (I) enhances the recording sensitivity of the heat-sensitive color-forming layer are not absolutely clear, but the following specific properties of the compound are considered to be a factor thereof. When melted, the melt of the compound of the formula (I) exhibits a relatively low viscosity and a high compatibility with the dye precursor and the color developing agent, and thus the dye precursor can easily react with the color developing agent in the melt, at a high reaction rate.

The absence of a lowering of the whiteness of the heat-sensitive color-forming layer is assumed to be due to the very low or substantially non-solubility in water of the compound of the formula (I).

Also, the substantial absence of the whitening phenomenon is assumed to be due to a very low or substantially non-sublimating property of the compound of the formula (I) at practical printing temperatures.

Furthermore, the high heat-stability of the heat-sensitive color-forming layer is due to a preferable melting point of the compound of the formula (I), which melting point is higher than a certain critical printing temperature.

The compound of the formula (I) can be produced by various synthetic methods; i.e., usually the compound can be easily produced by the Ullmann reaction and at a high yield in accordance with the following reactions:



wherein X represents a halogen atom, for example, a chlorine, bromine or iodine atom.

Usually, the sensitizing agent of the present invention is present in an amount of 10 to 1000% by weight, preferably 50 to 300% by weight, based on the weight of the color-forming agent.

The heat-sensitive color-forming layer of the present invention contains a substantially colorless dye precursor, preferably in an amount of 5 to 20% by weight.

The substantially colorless dye precursor comprises at least one leuco basic dye which can be selected from usual leuco basic dyes usable for the conventional heat-

sensitive color developing layer, for example, crystal violet lactone,

- 3-(N-ethyl-N-isopentylamino)-6-methyl-7-anilinofluorran,
- 5 3-diethylamino-6-methyl-7-anilinofluorran,
- 3-diethylamino-6-methyl-7-(o-, and p-dimethylanilino)-fluorans,
- 10 3-(N-ethyl-p-toluidino)-6-methyl-7-anilinofluorran,
- 3-pyrrolidino-6-methyl-7-anilinofluorran,
- 3-dibutylamino-6-methyl-7-anilinofluorran,
- 3-(N-cyclohexyl-N-methylamino)-6-methyl-7-anilinofluorran,
- 3-diethylamino-7-(o-chloroanilino)fluorran,
- 3-diethylamino-7-(m-trifluoromethylanilino)fluorran,
- 3-diethylamino-6-methyl-7-chlorofluorran,
- 3-diethylamino-6-methylfluorran, and
- 3-cyclohexylamino-6-chlorofluorran.

The color developing agent is usually present in an amount of 10 to 40% by weight in the heat-sensitive color-forming layer, and can be selected from conventional color developing agents.

Preferably, the color-developing agent usable for the present invention comprises at least one member selected from the group consisting of phenol compounds and organic acid compounds, for example, bisphenol A, benzyl p-hydroxybenzoate (Japanese Unexamined Patent Publication No. 52-140,483), bisphenol S, 4-hydroxy-4-isopropoxydiphenylsulfone (Japanese Unexamined Patent Publication No. 60-13852), 1,1-bis(4-hydroxyphenyl)cyclohexane and 1,7-bis(hydroxyphenylthio)-3,5-dioxaheptane (Japanese Unexamined Patent Publication No. 59-52694).

The heat-sensitive color-forming layer of the present invention contains a binder in an amount of 5% to 20% by weight. The binder can be selected from conventional binders and preferably comprises at least one member selected from the group consisting of water-soluble polymeric materials, for example, polyvinyl alcohols having various molecular weights; starch and derivatives thereof; cellulose derivatives, for example, methoxycellulose, carboxymethylcellulose, methylcellulose and ethylcellulose; and water-soluble synthetic polymeric materials, for example, sodium polyacrylate, polyvinylpyrrolidone, acrylamide-acrylic acid ester copolymers, acrylamide-acrylic acid ester-methacrylic acid terpolymers, styrene-maleic anhydride copolymer sodium salts, polyacrylamide, sodium alginate, geratine, and casein; and latexes of water-insoluble polymeric materials, for example, polyvinyl acetate, polyurethane, styrene-butadiene copolymers, polyacrylic acid, polyacrylic acid esters, vinyl chloride-vinyl acetate copolymers, polybutyl methacrylate, ethylene-vinyl acetate copolymers and styrene-butadiene-acrylic monomer copolymers.

The heat-sensitive color-forming layer of the present invention optionally contains an additional heat fusible sensitizing agent consisting of at least one conventional heat-fusible substance having a melting point of from 80° C. to 110° C., for example, the compounds disclosed in the Description of the Related Art of this specification. The additional sensitizing agent is preferably contained in an amount of 5 to 20%, based on the weight of the color developing agent.

The heat-sensitive color-forming layer of the present invention optionally contains 10 to 50% by weight of a white pigment comprising fine particles of at least one member selected from inorganic pigments, for example,

calcium carbonate, silica, zinc oxide, titanium dioxide, aluminum hydroxide, zinc hydroxide, barium sulfate, clay, calcined clay, talc, and surface-treated calcium carbonate and silica; and organic pigments, for example, urea-formaldehyde resins, styrene-methacrylic acid copolymers, and polystyrene.

The heat-sensitive color-forming layer of the present invention optionally contains 5 to 30% by weight of a wax substance which can be selected from conventional wax materials, and preferably, comprises at least one member selected from, for example, paraffin materials, amide type wax materials, bis-imide type wax material, and metal salts of higher fatty acids.

Usually, the heat-sensitive color-forming layer of the present invention is preferably in a dry weight of 1 to 15 g/m<sup>2</sup>, more preferably 2 to 10 g/m<sup>2</sup>.

In the heat-sensitive recording material of the present invention, the heat-resistive color-forming layer is formed on at least one surface of a substrate sheet.

The substrate sheet comprises a paper sheet, a coated paper sheet in which a paper substrate sheet is coated with a mixture of an inorganic or organic pigment and a binder, a laminated paper sheet in which a paper substrate sheet is laminated with at least one heat-fusible resinous film, for example, polyethylene or polypropylene film, a synthetic paper sheet consisting essentially of a plastic resin, or a plastic resin film. The substrate sheet preferably has a weight of 30 to 200 g/m<sup>2</sup>.

The heat-sensitive recording material of the present invention is prepared by coating at least one surface of the substrate sheet with a coating liquid comprised of the dye precursor, color developing agent, sensitizing agent, binder and optionally at least one additive, for example, a white pigment or wax substance, dissolved or dispersed in a volatile solvent, for example, water, and drying the resultant coating liquid layer on the substrate sheet.

## EXAMPLES

The present invention will be further explained by way of specific examples, which are representative and do not in any way restrict the scope of the present invention.

### SYNTHESIS EXAMPLE

#### Preparation of 1,2-diphenoxylbenzene

Potassium salt of phenol was prepared by mixing 42.3 g of phenol into 50 ml of toluene, and adding 25.2 g of potassium hydroxide to the resultant mixture while 50 vigorously stirring. Thereafter, the toluene was completely distilled away from the resultant potassium phenolate mixture under atmospheric pressure, and water was eliminated from the mixture by an azeotropic distillation procedure. The residue was mixed with 20 ml of pyridine and the mixture was subjected to refluxing. Then to the mixture was added 35.4 g of o-dibromobenzene and a small amount of a catalyst consisting of copper powder, and the resultant mixture was subjected to a reaction for 24 hours while refluxing pyridine. The 60 resultant reaction product was extracted with ether, and the resultant ether phase was washed with an alkali aqueous solution, an acid aqueous solution and then water, dried with a desiccant and then filtrated, and thereafter, the ether was distilled away from the filtrated product. The resultant crude product was recrystallized by ethyl alcohol. The refined product was in an amount of 24.0 g and exhibited a melting point of 92° C.

It was confirmed by nuclear magnetic resonance spectrometry and mass spectrometry that the refined product was 1,2-diphenoxylbenzene of the formula (I).

#### EXAMPLE 1

A heat-sensitive recording paper sheet was produced by the following procedures.

##### (1) Preparation of dye precursor dispersion A

A mixture having the composition as shown below was prepared.

| Component                                              | Amount<br>(part by wt) |
|--------------------------------------------------------|------------------------|
| 3-(N-isopentyl-N-ethylamino)-6-methyl-7-anilinofluoran | 20                     |
| 10% polyvinyl alcohol aqueous solution                 | 10                     |
| Water                                                  | 70                     |

The mixture was placed in a sand grinder to pulverize the dye precursor particles to a size of 1 μm or less, and a dispersion A was obtained.

##### (2) Preparation of color developing agent dispersion B

A mixture having the composition indicated below was prepared.

| Component                              | Amount<br>(part by wt) |
|----------------------------------------|------------------------|
| 4,4'-isopropylidenebiphenol            | 10                     |
| 1,2-diphenoxylbenzene                  | 10                     |
| 10% polyvinyl alcohol aqueous solution | 10                     |
| Water                                  | 70                     |

The mixture was placed in a sand grinder to pulverize the color developing agent particles to a size of 1 μm or less, and a dispersion B was obtained.

##### (3) Formation of heat-sensitive color-forming layer

A coating liquid was prepared by mixing 40 parts by weight of the dye precursor dispersion A, 160 parts by weight of the color developing agent dispersion B, 40 parts by weight of calcium carbonate pigment, 20 parts by weight of 30% paraffin aqueous emulsion, and 180 parts by weight of a 10% polyvinyl alcohol aqueous solution while stirring. The resultant coating liquid was coated on a surface of a paper sheet having a base weight of 50 g/m<sup>2</sup> to an extent such that, after drying and solidifying, the resultant dry coating layer was in a weight of 7.0 g/m<sup>2</sup>, the coated liquid layer was dried to form a heat-sensitive color-forming layer, and thus a heat-sensitive recording paper sheet was obtained.

The recording paper sheet was treated by a super calender to smooth the surface of the heat-sensitive color developing layer until it exhibited a Beck smoothness of 600 to 1000 seconds.

The calendered recording paper sheet was subjected to the following tests.

##### (1) Measurement of recording sensitivity and whiteness of colored image-free portion of the recording paper sheet

A test piece of the recording paper sheet was locally heated at a temperature of 120° C. under a pressure of 2.5 kg/cm<sup>2</sup> for 100 m seconds, using a heat inclination tester (made by Toyo Seiki Co.), and the darkness of the resultant colored image was measured by a color darkness tester (available under a trademark of Macbeth Darkness Tester RD-914, from Kollmorgen Co.). The recording sensitivity of the test piece was represented by the measured value of the color darkness. Preferably, the measured darkness was 1.20 or more.

Also, the darkness (whiteness) of a portion of the test piece free from the colored image was measured in the same manner as mentioned above. The whiteness of the test piece before the colored image-formation was represented by the measured value of the darkness. The 5 lower the measured darkness, the higher the whiteness of the test piece. Preferably the measured darkness was 0.12 or less.

(2) Measurement of heat stability

In the above-mentioned heat inclination tester, a test 10 piece was heated at a temperature of 70° C. under a pressure of 2.5 kg/cm<sup>2</sup> for 5 seconds. The color development under the above-mentioned conditions refers to a static color development at 70° C. The darkness of the colored image was measured in the same manner as 15 mentioned above.

The heat stability of the test piece at 70° C. was represented by the measured value of the darkness of the colored image. The lower the darkness, the higher the 20 heat stability of the test piece, and preferably, the measured value of the darkness was 0.2 or less.

(3) Resistance to whitening phenomenon

A test piece was heated at a temperature of 150° C., 25 using the above-mentioned heat inclination tester, to form a colored image.

The colored image-formed portion was left to stand for 24 hours at a temperature of 40° C. and a relative 30 humidity of 90%. Thereafter, the surface of the colored image was observed by the naked eye and evaluated as follows.

| Indication | Notification                        |
|------------|-------------------------------------|
| Good       | No whitening phenomenon observed    |
| Bad        | Clear whitening phenomenon observed |

The results of the tests are indicated in Table 1.

EXAMPLE 2

The same procedures as in Example 1 were carried 40 out with the following exceptions.

(1) Preparation of a pigment-coated paper sheet

An aqueous dispersion was prepared by dispersing 85 parts by weight of calcined clay in 320 parts by weight of water and was mixed with 40 parts by weight of a 45 50% aqueous emulsion of a styrene-butadiene copolymer and 50 parts by weight of a 10% aqueous solution of oxidized starch, to provide a pigment coating liquid.

A surface of a paper sheet having a base weight of 48 g/m<sup>2</sup> was coated with the pigment coating liquid and the resultant pigment coating liquid layer was dried to 50 form a dry pigment coating layer having a weight of 7.0 g/m<sup>2</sup>.

(2) Formation of color-forming layer

A coating liquid was prepared by mixing 50 parts by 55 weight of the dye precursor dispersion A, 200 parts by weight of the color developing agent dispersion B, 25 parts by weight of calcium carbonate, 20 parts by weight of a 30% aqueous emulsion of paraffin, and 180 parts by weight of a 10% aqueous solution of polyvinyl alcohol, and stirring the mixture.

The coating liquid was applied to the pigment-coated 65 surface of the paper sheet and the resultant coating liquid layer was dried to form a heat-sensitive color developing layer having a dry weight of 5.0 g/m<sup>2</sup>. The resultant heat sensitive recording paper sheet was subjected to the same tests as in Example 1.

The test results are shown in Table 1.

COMPARATIVE EXAMPLE 1

The same procedures as in Example 1 were carried out except that, in the preparation of the color developing agent dispersion B, 1,2-diphenoxylbenzene was replaced by stearyl amide.

The test results are shown in Table 1.

COMPARATIVE EXAMPLE 2

The same procedures as in Example 2 were carried out except that, in the preparation of the color developing agent dispersion B, 1,2-diphenoxylbenzene was replaced by stearyl amide.

The test results are shown in Table 2.

COMPARATIVE EXAMPLE 3

The same procedures as in Example 2 were carried out except that, in the preparation of the color developing agent dispersion B, 1,2-diphenoxylbenzene was replaced by phenyl 1-hydroxy-2-naphthoate.

The test results are shown in Table 2.

COMPARATIVE EXAMPLE 4

The same procedures as in Example 2 were carried out except that, in the preparation of the color developing agent dispersion B, 1,2-diphenoxylbenzene was replaced by 1,4-diphenoxylbenzene having a melting point of 75° C.

The test results are shown in Table 2.

COMPARATIVE EXAMPLE 5

The same procedures as in Example 2 were carried out except that, in the preparation of the color developing agent dispersion B, 1,2-diphenoxylbenzene was replaced by 1,3-diphenoxylbenzene having a melting point of 49° C.

The test results are shown in Table 2.

TABLE 1

| Example No. | Item | Recording sensitivity (D) | Whiteness (D) | Heat stability at 70° C. (D) | Whitening resistance |
|-------------|------|---------------------------|---------------|------------------------------|----------------------|
| Example     | 1    | 1.20                      | 0.07          | 0.10                         | Good                 |
|             | 2    | 1.25                      | 0.07          | 0.10                         | Good                 |
| Comparative | 1    | 0.92                      | 0.12          | 0.18                         | Good                 |
|             | 2    | 1.01                      | 0.12          | 0.15                         | Good                 |
| Example     | 3    | 1.25                      | 0.09          | 0.14                         | Bad                  |
|             | 4    | 1.22                      | 0.10          | 0.36                         | Good                 |
|             | 5    | 1.18                      | 0.80          | 1.15                         | Good                 |

Table 1 clearly shows that the heat-sensitive recording paper sheets of the present invention exhibited an excellent recording sensitivity, a satisfactory whiteness of a colored image-free portion thereof, even after colored image formation, a superior heat stability at 70° C., and a satisfactory resistance to the whitening phenomenon, whereas each of the comparative recording paper sheets of Comparative Examples 1 and exhibited an unsatisfactory recording sensitivity, whiteness, and heat stability at 70° C., that of Comparative Example 3 had a very poor whitening resistance, that of Comparative Example 4 exhibited a poor heat stability at 70° C., and that of Comparative Example 5 had a very poor whiteness and heat stability at 70° C.

We claim:

1. A heat-resistant recording material comprising: a substrate sheet, and

a heat sensitive color-forming layer formed on at least one surface of the substrate sheet and comprising a substantially colorless dye precursor, a color-developing agent reactive with the dye precursor upon heating to develop a color, and a binder, said heat-sensitive color-forming layer further comprising a sensitizing agent consisting essentially of 1,2-diphenoxylbenzene of the formula (I):



2. The heat-sensitive recording material as claimed in claim 1, wherein the dye precursor is present in an amount of from 5 to 20% by weight in the heat-sensitive color-forming layer.

5 3. The heat-sensitive recording material as claimed in claim 1, wherein the color-developing agent is present in an amount of from 10 to 40% by weight in the heat-sensitive color-forming layer.

4. The heat-sensitive recording material as claimed in 10 claim 1, wherein the binder is present in an amount of from 5 to 20% in the heat sensitive color-forming layer.

5 5. The heat-sensitive recording material as claimed in claim 1, wherein the sensitizing agent is present in an amount of 10% to 1000% based on the weight of the 15 color developer in the heat-sensitive color-forming layer.

6. The heat-sensitive recording material as claimed in 20 claim 1, wherein the heat-sensitive color-forming layer is in a dry weight of from 1 to 15 g/m<sup>2</sup>.

\* \* \* \* \*

20

25

30

35

40

45

50

55

60

65